

# UNITED STATES PATENT OFFICE.

IGNAZ KREIDL, OF VIENNA, AUSTRIA-HUNGARY.

## OPAQUING AGENTS FOR THE PRODUCTION OF WHITE ENAMELS.

1,150,772.

Specification of Letters Patent. Patented Aug. 17, 1915.

No Drawing.

Application filed September 4, 1913. Serial No. 788,112.

*To all whom it may concern:*

Be it known that I, IGNATZ KREIDL, a subject of the Emperor of Austria-Hungary, residing in Vienna, Austria-Hungary, have 5 invented certain new and useful Improved Opaquing Agents for the Production of White Enamels, of which the following is a specification.

This invention has for its object to produce improved opaquing agents for the production of white enamel more especially zirconium enamels and an improved process for the manufacture of such opaquing agents.

Zirconium compounds, tin compounds, titanium compounds and aluminium compounds have already been proposed for use as opaquing agents for white enamel. It has also been proposed to start from the alkali compounds of the metallic oxides for the 20 manufacture of such opaquing agents, and to remove the whole or part of the alkali by means of acids. Those processes are more particularly suitable for the manufacture of opaquing agents containing alkali, when it 25 is desired that the opaquing agents shall be obtained combined with a portion of the alkali, that is to say, where the alkali is to be removed only in part.

For the purpose of manufacturing such 30 opaquing agents and more especially opaquing agents free from alkali, there may be used in addition to the alkali compounds, also the acid compounds or the salts of those metallic oxides which are suitable for opaquing purposes. In these cases the acid is removed for instance by means of alkali.

When using acid compounds or non-heat refractory *i. e.* volatile salts, for instance sulfates, nitrates, salts of organic acids and 40 the like for the manufacturing of the opaquing agents free from alkali the acid may be eliminated directly by heating to a glow heat.

It has been observed in the manufacture 45 of opaquing agents according to the herein-before mentioned processes, that the opaquing effect is not so good when the salts formed by the chemical re-arrangement have been wholly eliminated, or the acid has been 50 completely removed.

Now I have discovered that the opaquing property of the product is increased by the presence of salts or acid.

The action of the salts or acids appears to 55 be connected with the colloidal character of the product and depends upon the fact that

the products which are to be used as opaquing agents are kept in a resistant state by the presence of the salts or of the acid.

The most favorable proportion of acid or 60 salts differs for each acid, but can be readily determined empirically. The said proportion is however limited in the upward direction, because a too great proportion of acid or salts causes the opaquing agent to lose 65 in opaquing power. When for instance an alkaline zirconium compound, such as a zirconate, is used for the manufacture of the opaquing agent, then according to this invention, the combined alkali is removed at 70 at least in part by means of an acid, preferably a weak acid. The alkali salt thus formed is removed by subsequent washing out only to the extent as to leave behind such a quantity of the said alkali salt which (as 75 found by experiment) will produce a favorable effect. These experiments are easily made, because for this purpose it is merely necessary to test the opaquing agent as to its covering power for various percentages of 80 salt. When once the most favorable percentage has been ascertained, it is an easy matter to determine by chemical means the stage at which the washing out operation must be stopped to retain the said ascertained percentage of salt. 85

In the manufacture of the improved opaquing agents from the alkali compounds it is to be understood that in the removal of the alkali by means of acids, acid may also 90 be combined, and then the excess of acid may be removed by heating to incandescence.

If an acid compound or a salt is used for the manufacturing of the opaquing agents the acid is removed at least in part by means 95 of alkali alone or alkali and heating to incandescence, and the washing out of the alkali salt is regulated in the same manner as hereinbefore stated.

In the manufacture of the improved 100 opaquing agents from acid compounds or salts, the washing out operation may be dispensed with, if the acid is eliminated directly by heating to incandescence alone. The acid, however, must not be eliminated completely, because the percentage of contained acid has a great influence upon the opaquing power. 105

I have discovered that acids or the salts of acids, such as organic acids which have a 110 low electrolytical dissociation are especially suitable for the purpose of this invention.

What is claimed is:

1. Opaquing agents for manufacturing white enamels comprising highly basic compounds or complexes, certain compounds of which have opaquing effects, containing a salt or salts of a volatile acid or acids.
2. Opaquing agents for manufacturing white enamels comprising a highly basic zirconium compound containing a salt or salts of a volatile acid or acids.
3. Opaquing agents for manufacturing white enamels comprising a highly basic compound containing zirconium oxid and a salt or salts of a volatile acid or acids.
4. Opaquing agents for manufacturing white enamels comprising a zirconium compound containing a salt or salts of an acid which relatively slightly ionizes.
5. An opaquing agent for manufacturing

white enamels comprising a compound of a 20 metal which produces opaquing effects, containing a small proportion of the radical or of a volatile acid or acids.

6. An opaquing agent for manufacturing white enamels comprising a compound of a 25 metal which produces opaquing effects, containing a small proportion of a radical or radicals of an acid which are relatively slightly ionized, such as the radical or radicals of organic acid.

In witness whereof, I have hereunto signed my name in the presence of two subscribing witnesses.

DR. IGNAZ KREIDL.

Witnesses:

HUGO REIK,  
AUGUST FUGGER.